

## UNITED STATES PATENT OFFICE

2,591,289

FROTHING AGENTS FOR USE IN  
FROTH FLOTATION PROCESSESRoger F. Powell, Gwelo, Southern Rhodesia, and  
Herbert Muggleton Stanley, Tadworth, Eng-  
landNo Drawing. Application October 12, 1949,  
Serial No. 121,054  
In the Union of South Africa, August 17, 1948

6 Claims. (Cl. 209—166)

1

This application is a continuation-in-part of our application Serial Number 112,842 filed on 27th August 1949, now abandoned.

This invention relates to froth flotation processes for the concentration of materials amenable to such processes, including the noble and base metal ores and their products, the non-metallic ores, coal and valueless materials which are selectively floated from valuable materials, in which processes froths are produced by the addition of frothing agents to the flotation pulp.

The invention consists in a process or processes utilising frothing agents in the same manner and for the same purpose as steam-distilled pine oil, but which by their nature need to be used in substantially smaller quantities than pine oil in order to produce closely similar results.

According to the invention in a froth flotation process, in addition to well-known promoting and collecting agents such as the xanthates et cetera there is present as frothing agent a tetra-alkoxy-paraffin having from two to five carbon atoms in the paraffin chain, a pair of alkoxy radicals—alkoxy being limited to methoxy, ethoxy, normal propoxy, or isopropoxy being attached (by the carbon-oxygen-carbon at "ether" linkage) to each terminal carbon atom of the chain. In any such tetra-alkoxy-paraffin the two pairs of alkoxy radicals need not necessarily be, though they may be, the same; for instance a pair of ethoxy radicals may be attached to one carbon atom and a pair of isopropoxy radicals attached to the other or another carbon atom, or there may be two pairs of ethoxy radicals or any similar combination of the four alkoxy radicals methoxy, ethoxy, normal propoxy, and isopropoxy.

The following examples serve to make quite plain the scope of the generalised structure described above:

## Example 1

1:1, 2:2 tetraethoxy-ethane



5

15

20

25

30

35

40

45

2

## Example 2

1:1, 4:4 tetramethoxy-butane



## Example 3

1:1 ethoxy-4:4 isopropoxy-butane



Carefully standardised laboratory flotation tests were carried out in a 2000-gram Denver-Fahrenwald fixed-speed flotation machine without the addition of any air other than that sucked in in the normal manner. Two different ores, each from a different mine, were tested: in each the valuable minerals to be floated were chalcopyrite and pyrrhotite, the latter only being auriferous. The two ores differed in the percentages of these minerals present, in their natural pH after grinding, and in the amount of deleterious colloidal material present. On each ore there was first done a "control test" using as frother "commercial triethoxybutane," whose properties have been established as superior to steam-distilled pine oil on several large well-known ore concentrators for several years.

## PROCEDURE ON FIRST ORE

2000 grams of moist ore was ground for 50 minutes in a ballmill with 1200 cubic centimeters of tap-water and 1.2 grams of copper-sulphate.

50 Pulp was washed out and made up to standard

volume in a 2000-gram Denver-Fahrenwald flotation machine.

0.10 grams of sodium-isopropyl-xanthate was then added to the pulp plus one drop from a standardised capillary tube, of the substance being tested as frother (each drop found by measurement to be approximately 0.0135 cc.). After 30 seconds the suction-air valve was opened, and a primary concentrate collected for exactly one hundred and twenty seconds. Suction-air valve was closed and another 0.25 grams of the xanthate added, plus 4 standardised capillary drops of the frother. Suction-air valve was opened, and froths allowed to run over the lip of the machine for 5 minutes, with a standard stream of water being meanwhile added to the pulp at the back of the machine. This constitutes the secondary concentrates. Suction-air valve was then closed, bottom plug was opened, and the tailings (residue) pulp washed out into a bucket. Primary concentrates, secondary concentrates, and tailings (residue) were filtered, dried at 100° cent., and analysed.

The pH of the tailings pulp was found to be approximately 9.2, the pulp being well-flocculated and the degree of grinding being approximately 62% minus 200-mesh.

#### PROCEDURE ON SECOND ORE

2000 grams of moist ore was ground for 35 minutes in a ballmill with 1200 cubic centimeters of tap-water. The pulp was washed out

and made up to standard volume in a 2000-gram Denver-Fahrenwald flotation machine.

0.10 grams of sodium-isopropyl-xanthate was then added to the pulp plus two drops (unless otherwise stated) from a standardised capillary tube, of the substance being tested as frother (each drop was found by measurement to be approximately 0.0135 cc.). After 30 seconds the suction-air valve was opened, and a primary concentrate collected for exactly one hundred and twenty seconds. Suction-air valve was then closed, another 0.25 grams of the xanthate added, plus 2 (unless otherwise stated) standardised capillary drops of the frother; suction air valve was opened, and froths allowed to run over the lip of the machine for 5 minutes, with a standard stream of water being added to the pulp at the back of the machine. This constitutes the secondary concentrate. Suction-air valve was closed, bottom plug opened, and the tailings (residue) pulp washed out into a bucket. Primary concentrates, secondary concentrates, and tailings (residue) were filtered, dried at 110° cent. and analysed.

The pH of the tailings pulp was found to be approximately 8.0 and the degree of grinding approximately 88% minus 100-mesh. Even after long standing, the water in the tailings pulp was very colloid-y. This particular ore notoriously gave rather low recoveries of the pyrrhotite, whatever frother was used (including pine oil).

The results of the tests were as follows:

#### FIRST ORE TESTED

| Substance tested as Frother                     | Product         | Product Percentage Weight of Ore | Mineral Grade of Product |                    |                          | Lbs. Valuable Mineral per ton of Ore |            |
|-------------------------------------------------|-----------------|----------------------------------|--------------------------|--------------------|--------------------------|--------------------------------------|------------|
|                                                 |                 |                                  | Percent Chalcopyrite     | Percent Pyrrhotite | Percent Valueless Gangue | Chalcopyrite                         | Pyrrhotite |
| Control Test: 1:1:3 Triethoxybutane Commercial. | 1st Conc.       | 8.17                             | 42.9                     | 38.8               | 18.3                     | 70.1                                 | 63.5       |
|                                                 | 2nd Conc.       | 6.71                             | 4.5                      | 63.8               | 31.7                     | 6.0                                  | 85.6       |
|                                                 | Combined Conc.  | 14.88                            |                          |                    |                          | 76.1                                 | 149.1      |
|                                                 | Residue         | 85.12                            | 0.14                     | 1.26               |                          | 2.4                                  | 33.5       |
|                                                 | Calculated Ore. | 100                              | 3.93                     | 9.13               |                          | 78.5                                 | 182.6      |
| 1:1:2:2: Tetraethoxyethane                      | 1st Conc.       | 7.44                             | 45.3                     | 39.6               | 15.2                     | 67.3                                 | 58.9       |
|                                                 | 2nd Conc.       | 7.09                             | 4.1                      | 64.1               | 31.8                     | 5.9                                  | 90.9       |
|                                                 | Combined Conc.  | 14.53                            |                          |                    |                          | 73.2                                 | 149.8      |
|                                                 | Residue         | 85.47                            | 0.07                     | 1.55               |                          | 1.2                                  | 26.4       |
|                                                 | Calculated Ore. | 100                              | 3.72                     | 8.81               |                          | 74.4                                 | 176.2      |
| 1:1:2:2: Tetraisopropoxyethane                  | 1st Conc.       | 9.87                             | 31.5                     | 44.7               | 23.8                     | 62.2                                 | 88.2       |
|                                                 | 2nd Conc.       | 11.23                            | 4.1                      | 35.0               | 60.9                     | 9.3                                  | 78.6       |
|                                                 | Combined Conc.  | 21.10                            |                          |                    |                          | 71.5                                 | 166.8      |
|                                                 | Residue         | 78.90                            | 0.14                     | 0.95               |                          | 2.2                                  | 15.0       |
|                                                 | Calculated Ore. | 100                              | 3.69                     | 9.09               |                          | 73.7                                 | 181.8      |
| 1:1:2:2: Tetra-n-Propoxyethane                  | 1st Conc.       | 9.18                             | 37.7                     | 41.7               | 20.6                     | 69.1                                 | 76.6       |
|                                                 | 2nd Conc.       | 7.22                             | 3.2                      | 55.2               | 41.7                     | 4.6                                  | 79.6       |
|                                                 | Combined Conc.  | 16.40                            |                          |                    |                          | 73.7                                 | 156.2      |
|                                                 | Residue         | 83.60                            | 0.12                     | 1.70               |                          | 2.0                                  | 28.5       |
|                                                 | Calculated Ore. | 100                              | 3.79                     | 9.24               |                          | 75.7                                 | 184.7      |

#### SECOND ORE TESTED

[From a different mine, but containing the same 2 minerals, in different proportions]

| Substance tested as Frother                        | Product         | Product Percentage Weight of Ore | Mineral Grade of Product |                    |                          | Lbs. Valuable Mineral per ton of Ore |            |
|----------------------------------------------------|-----------------|----------------------------------|--------------------------|--------------------|--------------------------|--------------------------------------|------------|
|                                                    |                 |                                  | Percent Chalcopyrite     | Percent Pyrrhotite | Percent Valueless Gangue | Chalcopyrite                         | Pyrrhotite |
| New Control Test 1:1:3 Triethoxybutane Commercial. | 1st Conc.       | 2.78                             | 18.8                     | 53.1               | 28.0                     | 10.5                                 | 29.6       |
|                                                    | 2d Conc.        | 5.47                             | 1.9                      | 59.8               | 38.3                     | 2.1                                  | 65.4       |
|                                                    | Combined Conc.  | 8.25                             |                          |                    |                          | 12.6                                 | 95.0       |
|                                                    | Residue         | 91.75                            | 0.04                     | 3.27               |                          | 0.7                                  | 59.9       |
|                                                    | Calculated Ore. | 100                              | 0.67                     | 7.74               |                          | 13.3                                 | 154.9      |
| 1:1:3:8: Tetraethoxypropane                        | 1st Conc.       | 4.07                             | 13.8                     | 57.3               | 28.0                     | 11.2                                 | 46.7       |
|                                                    | 2nd Conc.       | 6.94                             | 1.7                      | 51.8               | 46.5                     | 2.4                                  | 71.9       |
|                                                    | Combined Conc.  | 11.01                            |                          |                    |                          | 13.6                                 | 118.6      |
|                                                    | Residue         | 88.99                            | 0.07                     | 2.07               |                          | 1.2                                  | 36.8       |
|                                                    | Calculated Ore. | 100                              | 0.74                     | 7.77               |                          | 14.8                                 | 155.3      |
| 1:1:5:5: Tetraethoxypropane                        | 1st Conc.       | 4.51                             | 12.2                     | 52.4               | 35.4                     | 11.0                                 | 47.3       |
|                                                    | 2nd Conc.       | 4.51                             | 1.1                      | 63.5               | 35.4                     | 1.0                                  | 57.3       |
|                                                    | Combined Conc.  | 9.02                             |                          |                    |                          | 12.0                                 | 104.6      |
|                                                    | Residue         | 90.98                            | 0.10                     | 1.85               |                          | 1.9                                  | 33.7       |
|                                                    | Calculated Ore. | 100                              | 0.69                     | 6.91               |                          | 13.9                                 | 138.3      |

NOTE.—Such a powerful frother that only half the standard quantities used.

We claim:

1. A process of concentrating material comprising subjecting the material to froth flotation in the presence of a collecting agent and a frothing agent consisting essentially of a tetra-alkoxy paraffin having in the paraffin chain from two to five carbon atoms, a pair of alkoxy radicals selected from the group methoxy, ethoxy, normal propoxy and iso-propoxy being attached to each terminal carbon atom in the chain.

2. A process of concentrating material comprising subjecting the material to froth flotation in the presence of a collecting agent and a frothing agent consisting of a bisacetal of ethane, propane, butane and pentane.

3. The process claimed in claim 1 in which the frothing agent is tetra-ethoxy-ethane.

10

15

4. The process claimed in claim 1 in which the frothing agent is tetra-ethoxy-propane.

5. The process claimed in claim 1 in which the frothing agent is tetra-ethoxy-pentane.

6. The process claimed in claim 2 in which the frothing agent is tetra-ethoxy-butane.

ROGER F. POWELL.

HERBERT MUGGLETON STANLEY.

#### REFERENCES CITED

The following references are of record in the file of this patent:

Richter's Organic Chemistry, second English edition, formulated by Percy E. Spielman, published by P. Blakiston's Son & Co., 1012 Walnut St., Philadelphia, Pa., vol. 1, pages 346-348.